

# United States Patent [19]

Deeg

[11] Patent Number: 4,954,605

[45] Date of Patent: \* Sep. 4, 1990

[54] AROMATIC POLYETHERKETONE FIBER PRODUCT

[75] Inventor: Martin H. G. Deeg, Maplewood, N.J.

[73] Assignee: Hoechst Celanese Corp., Somerville, N.J.

[\*] Notice: The portion of the term of this patent subsequent to Apr. 4, 2006 has been disclaimed.

[21] Appl. No.: 332,532

[22] Filed: Mar. 31, 1989

### Related U.S. Application Data

[60] Division of Ser. No. 107,845, Oct. 6, 1987, Pat. No. 4,849,148, which is a continuation of Ser. No. 732,537, May 10, 1985, abandoned.

[51] Int. Cl.<sup>5</sup> C08G 8/02; C08G 65/38; D02G 3/00; D01F 1/00

[52] U.S. Cl. 528/125; 528/126; 528/128; 528/219; 264/176.1; 264/211.22; 264/205; 428/364

[58] Field of Search 528/125, 126, 128, 219; 264/176.1, 211.22, 205; 428/364

### References Cited

#### U.S. PATENT DOCUMENTS

4,320,224 3/1982 Rose et al. .... 528/219  
4,360,630 11/1982 Smith ..... 528/125

#### FOREIGN PATENT DOCUMENTS

57-191322 11/1982 Japan .

#### OTHER PUBLICATIONS

Ali et al., "Spinning and Drawing of Polyetheretherketone (PEEK)"

tone (PEEK)", Research Disclosure 216, 104-5 (Apr. 1982).

Xu et al., "Poly (ether-ether-ketone): Melt Spinning and Fiber Properties," Sen-I Gakkaishi 41 (1):59-65 (1985) (English translation provided).

Primary Examiner—Morton Foelak

Assistant Examiner—P. Hampton-Hightower

Attorney, Agent, or Firm—Marvin Tucker

### [57] ABSTRACT

Filaments are produced from polymers having an inherent viscosity of at least 0.7 measured in concentrated sulfuric acid and containing in the polymer chain at least 50 percent of the repeating units.



by melting the polymer and heating the melt to a temperature of from about 20° C. to about 80° C. above the melting point of the polymer, passing the melt through a filter pack having a filtering area of at least about 8 in<sup>2</sup> and a total volume of at least about 1.2 in<sup>3</sup> per pound of polymer extruded per hour, and containing inert, irregularly shaped particles having a mesh size of about 25 to 140 to provide a pressure drop at least about 800 psig., and extruding the melt through spinning openings of desired shape to form filaments. The process is capable of producing fibers and yarns having a dpf of about 15 to 100, a tenacity of about 1 to 2 grams per denier, an elongation at break of about 50 to 160 percent and a modulus of about 20 to 30 grams per denier.

3 Claims, 1 Drawing Sheet





## AROMATIC POLYETHERKETONE FIBER PRODUCT

## CROSS REFERENCE TO RELATED APPLICATIONS

This application is a divisional of application Ser. No. 107,845, filed Oct. 6, 1987 U.S. Pat. No. 4,849,148 which is a continuation of application Ser. No. 732,537, filed May 10, 1985, and now abandoned.

This invention relates to filaments and fibers of a certain class of aromatic polyetherketones and their production by a melt spinning process.

## BACKGROUND OF THE INVENTION

The polymers contemplated by this invention are disclosed in the U.S. Pat. Nos. 4,320,224; 4,360,630; and 4,446,294 the entire disclosures of which are incorporated by reference. These crystalline, linear polymers contain in the polymer chain at least 50 percent of the following repeating unit (hereinafter referred to as "repeating unit I"):



The polymers may be composed solely of repeating units I or may contain other repeating units as hereinbefore defined and they have inherent viscosities IV (measured at 25° C. in a solution of the polymer in concentrated sulphuric acid of density 1.84 g cm<sup>3</sup>, said solution containing 0.1 g of polymer per 100 cm<sup>3</sup> of solution) of at least 0.7. These polymers are exceptionally useful in that they possess excellent mechanical and electrical properties, coupled with outstanding thermal and combustion characteristics. They also show resistance to a very wide range of solvents and proprietary fluids. They are thus very suitable in applications where the service conditions are too demanding for the more established, high performance polymers and in particular where the polymers are liable to high service temperatures.

In view of the foregoing desirable properties of these particular aromatic polyetherketones, it would be advantageous if they could be easily formed into filaments and fibers since the latter products could then be made for example into knitted, woven and non-woven fabrics, fiberfill and insulation products suitable for applications utilizing their excellent physical and chemical properties. However, the same combination of properties which would make filaments and fibers made from these polymers very desirable in various applications, e.g. heat and solvent resistance, also cause them to be very difficult to spin into such filaments and fibers. Thus, if it is attempted to melt spin these polymers into filaments in a conventional manner, the use of a relatively low spinning temperature results in a high melt viscosity which significantly reduces spinning stability due to high spinning pressures, clogging of the spinneret holes, uneven polymer coagulation and frequent filament rupture. On the other hand, unduly high spinning temperatures result in polymer degradation and cross-linking which cause void, gel and speck formation in the filaments and render them unsuitable for most uses. In view of these factors, successful spinning into filaments of the polymers contemplated by this invention is not easily

accomplished. Although U.S. Pat. Nos. 4,320,224, and 4,446,294 disclose broadly that polymers containing a major proportion of repeating unit I may be fabricated into any desired shape including fibers, they do not have any specific teaching of how such fibers may in fact be formed.

## BRIEF DESCRIPTION OF THE DRAWINGS

The FIGURE drawing discloses a spinning apparatus 10 wherein polymer chip (s) denoted by (1) fed to a closed hopper under nitrogen or vacuum, whereto passed into a screw extruder denoted by (2) thereby heated by electrical heater bands divided into three zones; (3) 15 denotes the polymer heated between 355° C. to 415° C. in the section of the extruder then melted and heated in the center and front sections, respectively; (4) denotes the polymer melt passed into the block spinning chamber and passed through a standard zenith gear pump denoted by (5) and back to the block spinning chamber denoted by (4). The polymer melt is passed through a filter pack denoted by (6) which contained shattered metal filtering medium denoted by (7); then the polymer melt is passed through a screen denoted by (8) and through the holes of the spinneret denotes by (9). The 20 polymer melt is then extruded into multifilaments denoted by (10) and collected into yarn at the yarn guide denoted by (11) and yarn is taken up in 5 to 10 wraps around a speed controlled take-up roll denoted by (12).

## SUMMARY OF THE INVENTION

In accordance with this invention, a linear aromatic polyetherketone comprising at least 50 percent of repeating unit I in the polymer chain and having an inherent viscosity (IV') of at least 0.7 as hereinbefore defined is melt spun at a temperature in the range of from about 20° C. above to about 80° C. above the melting point of the polymer, using a filter pack filtering area of at least about 8 in<sup>2</sup> preferably about 15 to 25 in<sup>2</sup> and a total volume of at least about 1.2 in<sup>3</sup>, preferably about 1.6 to 2.3 in<sup>3</sup> per pound of polymer extruded per hour with a filtering medium of inert particles having numerous angles, indentations and/or irregularities and a mesh size of about 25 to 140. The particles of filter medium may be for example "shattered metal" e.g. carbon steels and stainless steels, aluminum oxides and silicates, e.g. sold under the trademarks "Alundum" and "Bauxilite", ground ceramics and sand.

The filter medium must be sufficient to provide a 50 pressure drop of at least about 800 psig., preferably about 950 to 3000 psig. Such a filter pack size and type of filter medium has been found to provide an adequate degree of shear necessary for stable spinning of the contemplated polymers to filaments of commercially acceptable deniers without an undesirably large increase in spinning pressure.

In addition to the filter medium mentioned previously, it is in most instances desirable to employ a fine filter screen across the filtering area downstream of the 60 filter for the purpose of separating specks and gels which get through the filter pack. Such a screen in general has openings of under about 20 microns, preferably in the range of about 3 to 10 microns.

In order to further maintain stable spinning in carrying out the process of the invention, it is preferable not to quench the filaments extruded from the spinneret holes, i.e. the filaments are cooled in non-circulating air at ambient temperatures and are not contacted with any

forced draft of any gas cooler than the surroundings. Moreover, to maintain stable spinning, it is preferable to operate the process such that the extruded filaments converge within about 15 to 50 inches preferably in the range of about 20 to 30 inches of the spinneret.

The remaining conditions which may be utilized in the process are conventional for melt spinning and are not considered critical to the invention. Thus the polymer may be extruded through a spinneret plate containing, for example 10 to 100 holes each with a diameter in the range of about 0.009 to 0.013 inch to produce filaments which are taken up at a speed, for example of about 70 to over 200 meters per minute. Such filaments each has a denier, for example in the range of about 15 to 100, preferably about 15 to 40. The filaments may have a circular cross-section resulting from the use of circular spinneret holes, or may have any of various non-circular cross-sections resulting from the use of different non-circular spinneret hole shapes, e.g. multilobal cross-sections containing, for example, six lobes, produced by using star-shaped spinneret holes containing, for example six protrusions.

The fibers and yarns resulting from the process of this invention generally have a tenacity in the range of about 1 to 2 grams per denier, an elongation at break of about 50 to 160 percent and modulus of about 20 to 30 grams per denier. The birefringence of the filaments is in the range of about 25 to 150.

The preferred polymers which may be formed into filaments in accordance with this invention consist solely of repeating unit I and have an IV of at least 0.7 measured in concentrated sulfuric acid as described previously. As disclosed in U.S. Pat. No. 4,320,224, such polymers may be made by polycondensing hydroquinone and 4,4'-difluorobenzophenone with an alkali metal carbonate or bicarbonate (excluding the sole use of sodium carbonate or bicarbonate) in a solvent such as diphenyl sulfone. Part of the 4,4'-difluorobenzophenone e.g. up to 50 percent, may be replaced with 4,4'-dichlorobenzophenone or 4-chloro-4'-fluorobenzophenone. These polymers consisting solely of repeating units I in the polymer chain generally have a melting point of about 335° C. to that in carrying out the spinning process of the invention, the polymer melt is extruded at temperatures of about 355° C. to about 415° C. Polymers containing up to 50 percent of repeating units other than repeating unit I are also contemplated and may be formed by replacing up to 50 mol percent of the hydroquinone in the monomer mixture with any of certain other dihydroxyphenols and up to 50 mol percent of the 4,4'-difluorobenzophenone with any or certain other aromatic dihalides. For example, up to 50 mol percent of the hydroquinone may be substituted with a dihydroxy phenol cocondensant of the formula:



in which A is a direct link, oxygen, sulphur,  $\text{SO}_2$ ,  $-\text{CO}-$ , or a divalent hydrocarbon radical. Examples of such bisphenols are:  
 4,4-dihydroxybenzophenone  
 4,4,40-dihydroxydiphenylsulphone  
 2,2'-bis-(4-hydroxyphenyl) propane  
 4,4'-dihydroxybiphenyl.

The substitution of part of the hydroquinone with any of the foregoing dihydroxy phenols causes the following repeating units (hereinafter referred to as "repeating unit II") to be present in the polymer chain interspersed with repeating unit I:



Alternatively or in addition to the substitution of part of the hydroquinone with another dihydroxyphenol, up to 50 mol percent of the 4,4'-difluorobenzophenone may be replaced with one or more dihalide cocondensants of the formula:



in which X and X', which may be the same or different, are halogen atoms and are ortho or para—preferably the latter—to the groups Q and Q'; and Q and Q', which may be the same or different, are  $-\text{CO}-$  or  $-\text{SO}_2-$ ; Ar' is a divalent aromatic radical; and n is 0, 1, 2 or 3.

The aromatic radical Ar' is preferably a divalent aromatic radical selected from phenylene, biphenylene or terphenyllylene.

Particularly preferred dihalides have the formula:



where m is 1, 2 or 3.

Examples of such dihalides include:

4,4-dichlorodiphenylsulphone  
 4,4-difluorodiphenylsulphone  
 4,4'-dichlorobenzophenone  
 bis-4,4'-(4-chlorophenylsulphonyl) biphenyl  
 bis-1,4-(4-chlorobenzoyl) benzene  
 bis-1,4-(4-fluorobenzoyl) benzene  
 4-chloro-4'-fluorobenzophenone  
 4,4'-bis-(4-fluorobenzoyl) biphenyl  
 4,4'-bis-(4-chlorobenzoyl) biphenyl.

Although substitution of the 4,4-difluorobenzophenone with 4,4'-dichlorobenzophenone and/or 4-chloro-4'-fluorobenzopheno does not change the units of the polymer chain, it has been found that up to 50 mol percent of the difluoro compound may be so replaced without adverse effects and with consequent cost advantage. Substitution of part of the 4,4-difluorobenzophenone with any of the other specified dihalides cause the following units (hereinafter referred to as "repeating unit III") to be present in the polymer chain



in which the oxygen atoms in the sub-units:



are ortho or para to the groups Q and Q'.

Where both dihydroxy phenol and dihalide (other than the dichloro- or chlorofluoro benzophenone) co-condensants are employed, the polymer will contain, in addition to repeating units I, II and III, the following repeating units (hereinafter referred to as "repeating unit IV"):



#### DESCRIPTION OF PREFERRED EMBODIMENTS

##### EXAMPLE 1

Filaments were produced in accordance with the process of this invention using spinning apparatus as depicted schematically in the drawing. Polymer chip in an amount of 1.3 lb/hr. with polymer chains consisting solely of repeating unit I having an inherent viscosity in concentrated sulfuric acid of 0.9 and prepared as described in Example 1 of U.S. Pat. No. 4,320,224, was fed to closed hopper 1 under nitrogen or vacuum. From there, it passed into screw extruder 2 which was heated by electrical heater bands divided into three zones. The polymer which followed the path indicated by line 3 was heated to 246° C. in the section of the extruder, and melted and heated to 346° C. and 363° C. in the center and front sections respectively. The melted polymer was then passed into the top of "block" i.e. spinning chamber, 4 from which it was passed to pump 5 (a standard Zenith gear pump) and back into block 4 which was surrounded by electrical heater bands. The polymer melt, heated in block 4 to about 382° C., was passed into filter pack 6 which contained shattered metal filtering medium 7 in which the particles had a mesh size of about 25 to 50. The filter pack had a filtering area of slightly over 20 in<sup>2</sup> and a total filter volume of about 2.75 in<sup>3</sup> or 2.12 in<sup>3</sup> per pound of polymer extruder per hour. The pressure drop of the polymer melt developed in the filter pack was about 1000 psig. At the start of spinning from filter pack 7, the polymer melt passed through screen 8 having openings less than 20 microns in size and thence through the 33 holes of spinneret 9 arranged in a circle in the spinneret plate. The holes each had a diameter of 0.0127 inch and a length of 0.019 inch. Filaments 10 extruded from the spinneret were collected into a yarn at yarn guide 11 located about 24 inches below the spinneret. The yarn was taken up without quenching in 5 to 10 wraps around speed controlled take up roll 12 at a speed of about 165 meters per

minute and was forwarded to a tension control winder (not shown).

The resulting yarn had a dpf of 18.1, a tenacity of 1.64 grams/denier, an elongation at break of 86 percent, a modulus of 25.97 grams/denier, and a birefringence of 86.

##### EXAMPLE 2

The process of Example 1 was followed except that the yarn was taken up on roll 12 at a speed of about 195 meters per minute.

The resulting yarn had a dpf of 15.0, a tenacity of 1.42 grams per denier, an elongation at break of 66 percent, a modulus of 25.01 grams per denier, and a birefringence of 110.

The yarn produced by the process of this invention may be subjected to a drawing treatment using techniques well-known in the art to increase its tenacity. Furthermore, the filaments and yarns produced by the disclosed process may be converted to other fiber products such as tow, staple fiber, staple spun yarn etc. by means of conventional methods.

The various fiber products which may be produced in accordance with the invention are suitable for a variety of end-uses requiring good high temperature performance. For example, they may be used in the preparation of high performance structural components, e.g. by blending with carbon fiber in the form of filament or staple spun yarns, knitting or weaving the blend into a fabric and heat pressing the fabric into the desired shape. The fibers of the invention may also be used as a component of filter bags used in hostile environments and, in the form of knitted or woven fabrics, in the manufacture of various textile products requiring resistance to high temperatures such as specialized clothing, draperies and upholstery fabrics, e.g., those employed in airline seats.

I claim:

1. Multifilament and yarns of a polymer having an inherent viscosity of at least 0.7 measured in concentrated sulfuric acid, said polymer containing in the polymer chain at least 50 percent of the repeating units:



50 said fibers and yarns having at least ten filaments and a dpf of about 15 to 100, a tenacity of about 1 to 2 grams per denier, an elongation at break of about 50 to 160 percent, and a modulus of about 20 to 30 grams per denier.

55 2. The yarns of claim 1 wherein said polymer consists solely of said repeating units in the polymer chain.

3. The fibers and yarns of claim 2 wherein the individual fibers having a birefringence of about 25 to 150.

\* \* \* \* \*